

## UNITED STATES PATENT OFFICE

AXEL VIGGO BLOM, OF GROSSHOECHSTETTEN, SWITZERLAND

## PIGMENTARY BASE PRODUCT AND PROCESS FOR MAKING THE SAME

No Drawing.

Application filed April 5, 1927. Serial No. 181,278.

My invention concerns a material adapted to serve as the pigmentary base for paints and particularly such paints as are suitable for use as rustproof coatings for iron and other objects and surfaces, and the process for the manufacturing the same. In particular my invention relates to a pigmentary base for which metallic lead either alone or in the form of alloys with a largely preponderating lead content serves as the starting material.

The object of my invention is to provide a new and improved material of this character, which has properties making it particularly suitable as a base for anti-corrosive paint purposes. My material is different in structure from material obtained for instance in the atomization of lead by mechanical means, where the product, though finely divided, consists so to speak of solid little drops. The structure of my product is on the contrary exceedingly porous and spongy, which brings about the important advantage that it is readily and perfectly penetrated by the vehicles, such as linseed oil and other materials, used for the purpose of preparing paints therefrom. Furthermore this spongy condition brings about a strong capacity of reacting with the fatty acids set free, for instance, from linseed oil, during the process of drying and by this means facilitates the production of a dense film of paint and furnishes very favorable conditions during the aging of the same.

Another advantage of my improved product is its extremely fine division, as the maximum size of the individual particles composing the same must not go above 50 microns. Owing to this high degree of dispersion, the covering power of paints made by using it as a base, is much greater than that of ordinary paints.

As far as the chemical composition of my product is concerned, I am of the opinion that the same consists of a fine dispersion of lead in lead oxide, or a pyrosol of lead in lead oxide, wherein the lead oxide in the disperse system constitutes the exterior phase, which surrounds the highly dispersed lead.

In carrying out the process of producing

my improved product I proceed in the following manner:

I have discovered that pigmentary bodies of particular activity are obtained when lead alloys, the melting points of which are lower than that of pure lead, are used as starting materials in place of metallic lead. These are slowly oxidized while being maintained at a temperature between the melting point of the alloy and that of pure lead. For instance, an alloy containing 85% of lead, 13% of antimony, and 2% of tin may be used, and this is introduced into a furnace of the usual construction provided with a flat pan-shaped hearth, the interior of which must be adapted to be closed air-tight, so that a slight vacuum can be established therein. I then melt the said metallic material, either by means of electricity, gas, or in any other suitable manner, so that the melted material spreads out in a thin layer upon the hearth. I then establish a vacuum of the desired degree in the interior of the said furnace and by means of the same cause air to be drawn into the furnace through a plurality of tuyères located in a suitable position above the melted bath, the outward ends of which tuyères are in communication with the atmosphere. The interior ends of the said tuyères are arranged in such a position above the melted bath that the air jets issuing from the said tuyères impinge upon the same and a vigorous motion of the air is induced locally.

The action of the air causes the formation of the pigmentary product described above, as a portion of the molten material oxidizes, while the rest is finely dispersed through the oxide, the whole thus forming the pyrosol mentioned above.

It is of importance that the temperature of the molten bath be closely regulated and watched and for this purpose the color of the pigmentary body must be carefully observed. If the pigment assumes a yellowish color, the temperature has been allowed to rise too high. In that case the heating is cut down or the amount of air sucked in is increased. The normal color which the pigment should have is dark gray.

When using an alloy of the composition

mentioned above, I have obtained good results by keeping the temperature of the molten bath between 250 and 280° C.

As the pigmentary body forms on the surface of the molten bath, as stated above, it is carried away by the suction of the air. It is collected in any suitable manner, such for instance in a bag plant similar to those used for the deposition of flue dust.

10 In the same ratio as the pigmentary product formed is sucked out of the furnace, fresh raw material is introduced therein so that the process becomes continuous.

As stated above, the maximum size of the 15 particles of the pigmentary body must not exceed 50 microns and material coarser than that is removed by air separation. Some-what coarser material may be brought to the required degree of fineness by grinding in a 20 ball mill or other suitable device. Residue too coarse for this treatment returns to the furnace for retreatment.

As the operation is carried out in a vacuum 25 no poisonous lead dust can escape into the work rooms and any leak is indicated by a rise in pressure.

Having thus described my invention what I claim as new and desire to secure by Letters Patent is:

30 1. A pigmentary base of the character described, comprising the product produced by the oxidation of a lead alloy containing substantially 85 percent lead, 13 percent antimony and 2 percent tin, said oxidation having been carried out at a temperature between 250° C. and 280° C.

2. A process for the production of a pigmentary base of the character described, 35 which consists in melting an alloy of lead containing at least 80 percent lead and having a melting point below that of pure lead, and oxidizing said alloy at a temperature between its melting point and the melting point of pure lead.

40 3. A process for the production of a pigmentary base of the character described, which consists in melting an alloy of lead containing substantially 85 percent lead, 13 percent antimony, and 2 percent tin, and oxidizing said alloy at a temperature between 50 250° C. and 280° C.

45 In testimony whereof, I have signed my name to this specification this twenty-third day of February, 1927.

55 AXEL VIGGO BLOM.